

## UNITED STATES PATENT OFFICE.

MARK RAY CONE, OF SUDBROOK PARK, MARYLAND, ASSIGNOR, BY MESNE ASSIGNMENTS, TO THE UNION TRUST COMPANY, OF CLEVELAND, OHIO, A CORPORATION OF OHIO.

## PROCESS OF TREATING BITUMINOUS MATERIAL.

No Drawing. Application filed October 24, 1921, Serial No. 510,129. Renewed August 2, 1928.

This invention relates to a process for the treatment of bituminous materials, for example, asphalt, pitch, hydrocarbon residues or mixtures thereof, to render the same completely miscible in water without the admixture of any emulsifying agents.

The invention relates particularly to an improved process whereby the bituminous material or substance, such as asphalt, pitch, hydrocarbon residues or mixtures thereof, may be stored for an indefinite period or transported from place to place in a condition which will permit the same to be spread while at ordinary atmospheric temperature upon the surface to be covered, such as a roof, a wall or a roadway in a layer or a plurality of layers of any desired thickness without local treatment by the application of heat or without any change whatever except the addition of a sufficient quantity of water to produce the desired flow of the material.

The invention consists broadly in treating a bituminous substance to subdivide the same into minute particles approximating to some extent a colloidal state, and then subjecting these particles to a treatment causing the same to set and harden in such a way that the particles will be of substantially uniform consistency throughout, so that the particles will not readily coalesce. The invention further consists in treating the bituminous material so that it may be transported for long distances and maintained for considerable periods of time in a semi-solid condition having a relatively small amount of additional weight by reason of the added moisture but which will be miscible with water at ordinary temperatures without further treatment and adapted to form layers of any desired thickness.

The invention further consists in providing a product in the form of a bituminous paste or cement that is semi-solid and plastic, capable of being maintained in this condition for indeterminate periods of time and of being spread in layers or formed into shapes in molds or dies, which will coalesce upon being subjected to distillation or evaporation to form a compact, coherent and durable substance possessing all the qualities inherent in the material from which it was originally formed.

Furthermore, the invention consists in the

new and novel details and features of operation and the novel combinations and arrangements of steps in the process for the treatment of bituminous substances herein-after set forth and claimed.

The bituminous substances to be treated such as asphalt, pitch, mineral oil residues and mixtures thereof, all of which are commonly grouped under the generic term of bitumen, are first heated to a temperature above the fusing point so as to convert the same to a relatively thin fluid. The material may then be passed through a sprayer or atomizer of any preferred or well known construction, which subdivides the same into a state of subdivision which with respect to the greater part of material handled approximates a colloidal state of coarse dispersion. These minute particles are then subjected to the action of a moving body of fluid—as, for example, to a current of air or a body of water in motion, whereby the particles are dispersed with a gradually increasing velocity which will further subdivide the same and normally prevent the same from coming into contact with each other. Preferably a current of air is employed having its movement continuous over a smooth surface and accelerated in a direction away from the point of spraying or atomization. In case a body of liquid is used, it may be caused to have a rotary movement within cylindrical confining walls and propelled by any suitable means such as a blade propeller which will give the central portion a greater velocity of rotation than the outer portion where the sprayed material may be supplied.

The fluid is maintained at a temperature below the fusing point of the material but well above the solidifying point, so that the cooling effect upon the particles during this step of the process will be relatively slow. For example, if the material is heated to a temperature of 180° F., then the dispersing fluid would be maintained approximately at 140° F.

After being subjected to the action of the dispersing fluid for a period of time sufficient to permit the surface of the particles to set or harden sufficiently to limit and prevent coalescence if brought into contact, the particles are then immersed in a non-solvent body of liquid, preferably water,

which is maintained at a temperature somewhat below the temperature of the dispersing fluid,—for example, at 120° F.

This liquid may be conducted to any suitable container, such as a settling tank or vat, and the contents allowed to cool slowly to atmospheric temperature. During this period the particles gradually settle out upon or toward the bottom of the tank leaving a quantity of supernatant liquid substantially free of particles, which is then removed. Subsequently an additional quantity of the liquid is drained off until the residue or precipitate is in a semi-liquid or a flocculent condition adapted to be transported and spread upon a surface to be covered.

As long as this product is kept in a moist condition, the particles on account of their character and previous treatment will not coalesce or coagulate but each particle will retain its identity and the mass as a whole will be readily miscible in water. If the mass is allowed to become dry, however, or if the material is spread in a layer and the water permitted to evaporate, the particles will coalesce to form a close, compact, coherent substance resembling in its physical and chemical characteristics the original material from which it was produced.

By means of this process I produce a product comprising bitumen in the form of very finely-divided particles which, so long as a minimum quantity of moisture remains adsorbed on the surface, will be stable throughout the range of ordinary atmospheric temperatures, which will readily coalesce, however, upon the removal of the moisture to form the characteristic bituminous material.

Such a product may be prepared at a central point and distributed throughout a wide area without requiring or employing plants for treatment or preparation at the place of local application, where it may be spread at normal temperature in one or more layers of desired thickness, either with or without admixture of sand, stone or fibrous material and without any modification or treatment except the addition of such

amount of water as may be required to give 50 the needed plasticity.

The process may be carried out by the adaptation of standard and well known forms of apparatus and may be practiced commercially for the treatment of either 55 large or small quantities of material.

Although I have shown and described and have pointed out in the annexed claims, certain novel features of my invention, it will be understood that various omissions, substitutions and changes in the several steps of my process and in its operation may be made by those skilled in the art without departing from the spirit of my invention.

Having thus described my invention, I 65 claim:

1. In the art of treating bituminous material to form a plastic mass, the process which consists in spraying the material at a temperature above the fusing point to subdivide the same into fine particles, preventing contact between the said particles until the surfaces thereof have cooled below the melting point, immersing said particles in heated water, cooling the same gradually to 75 normal atmospheric temperature and removing the water until the material forms a moist, plastic paste.

2. The process of treating bituminous material to form a plastic substance capable of being spread cold in a thin layer at normal temperature as a surface coating which consists in spraying the melted bituminous material into a moving body of fluid to hold the particles out of contact with each other and harden the surfaces of the same, slowly cooling the particles with water and allowing the particles to settle as a flocculent paste, removing the excess water, spreading the paste over a surface and permitting the adsorbed liquid to evaporate, thereby to form a dense, homogeneous coating impervious to water.

Signed at Pikesville, in the county of Baltimore and State of Maryland, this 12 day 95 of Oct., A. D. 1921.

MARK RAY CONE.